

Oct. 20, 1925

1,557,672

H. A. DOERNER

CENTRIFUGAL CONCENTRATOR

Filed March 14, 1924

2 Sheets-Sheet 1

Fig. 1.



INVENTOR.  
Henry A. Doerner  
BY  
Pennie, Davis, Marvin, & Edmonde  
ATTORNEYS

Oct. 20, 1925.

1,557,672

H. A. DOERNER

## CENTRIFUGAL CONCENTRATOR

Filed March 14, 1924

2 Sheets-Sheet 2

Fig. 3.



Fig. 2.



## INVENTOR

INVENTOR  
Henry A. Doerner

9

BY  
Rennie, Davis, Marvin, & Edmonds

## ATTORNEYS

## UNITED STATES PATENT OFFICE.

HENRY ALFRED DOERNER, OF RENO, NEVADA.

## CENTRIFUGAL CONCENTRATOR.

Application filed March 14, 1924. Serial No. 699,216.

*To all whom it may concern:*

Be it known that I, HENRY A. DOERNER, a citizen of the United States, residing at Reno, in the county of Washoe, State of Nevada, have invented certain new and useful Improvements in Centrifugal Concentrators; and I do hereby declare the following to be a full, clear, and exact description of the invention, such as will enable others skilled in the art to which it appertains to make and use the same.

This invention relates to centrifugal concentrators and its object is to provide an improved method of and apparatus for separating finely divided solids of different densities in a continuous operation and by the action of centrifugal force. The invention is especially adapted for the concentration of values in crushed ores, slimes and similar materials.

The application of centrifugal action to the separation of finely divided solids of different densities, such as the concentration of ores, has frequently been suggested and tried in the past. So far as I am aware, these prior centrifugal separators or concentrators have not encountered much success or favor in the industrial arts. My present invention aims to provide an improved method of and apparatus for the application of centrifugal action to the separation of finely divided solids of different densities, in a continuous operation.

In accordance with the present invention, the finely divided solids of different densities, such as an ore, to be separated or concentrated, are subjected to the action of centrifugal force while suspended in a fluid, such as water, having a flow substantially opposite in direction to the direction of the centrifugal force. The solids of lower specific gravity are carried to an overflow by the fluid current, while the solids of higher specific gravity, on account of their greater response to centrifugal action, travel against the flow of the fluid current and are continuously discharged. The solids of higher specific gravity are continuously removed from the region of separation by an automatically operating liquid seal, such as a mercury seal. The solids of lower specific gravity are also continuously removed from the separating region.

The invention will be more readily under-

stood by reference to the accompanying drawings taken in conjunction with the following description. The drawings illustrate an apparatus particularly adapted for the practice of the invention. In the drawings,

Fig. 1 is an elevation mostly in section; Fig. 2 is a detail sectional view of a portion of the apparatus; and

Fig. 3 is a detail sectional view taken along the line 3—3 of Fig. 1.

Referring to the drawings, the apparatus there illustrated comprises a base 5 bolted or otherwise appropriately secured to a foundation 6. A hollow vertical shaft 7 is mounted in the base 5. A hub 8 is supported by ball-bearings 9 and is mounted to rotate about the shaft 7 as an axis. Appropriate lubrication for the revolving parts is provided by a pipe 10. A bevel gear 11 is keyed to the hub 8 and meshes with a companion bevel gear 12 secured to a shaft 13 appropriately driven from any suitable source of power.

The hub 8 carries a horizontal circular bottom plate 14 which may be integral therewith or otherwise appropriately secured thereto. A plurality of hollow annular members 16 are superposed in spaced relation above the circular bottom plate 14. These members 16 are mounted on vertical rods 17 and are held in spaced relation by a second series of annular members 18 and spacing blocks 19 similarly mounted on the rods 17.

The interior of the hollow annular members 16 is divided into a number of chambers or compartments 20 by partitions 21 (see Figs. 2 and 3). Each chamber 20 is connected to an independent fluid supply pipe 22 leading from a common distributing manifold 23. A plurality of relatively small holes 24 lead from each chamber 20 to the bottom face of the annular member 16; the holes 24 extending in a direction substantially parallel with the downwardly and inwardly flaring inner face of the annular member 16.

The annular members 18 have downwardly and inwardly flared aprons 18'. A series of upwardly and outwardly flared annular members 25 are bolted (at 26) to the tops of the hollow annular members 16, near the inner edge thereof. The three annular members 16, 18 and 25 are so positioned that an

annular downwardly and inwardly extending passage 27 is provided between the apron 18' and the member 25, while an annular horizontally extending passage 28 is provided beneath the inner half of the bottom face of the annular member 16.

The passages 27 and 28 form jointly a U-shaped conduit in which the discharge of the product or concentrate of higher specific gravity is effected by means of balanced forces. The bottom or lower end of each passage 27 communicates with the inner end of an annular discharge compartment 29. The outer side or face of each of the discharge compartments 29 is open and communicates with an independent launder or hopper 30.

A spider frame 31 is mounted on the rods 17 above the uppermost annular member 16. The spider frame 31 supports a central feed pipe 32 and the distributing manifold 23 which surrounds the feed pipe. A plurality of grooves 33 in the upper portion of the wall of the manifold 23 are connected to pipes 34 adapted to supply a liquid of high specific gravity, such as mercury, to points opposite each of the passages 28. The feed pipe 32 may be utilized for supplying the liquid of high specific gravity (such as mercury) to the lowermost passage 28.

The bottom plate 14 and the superposed annular members (16, 18 and 25) together with their appurtenances constitute the rotatable element of the apparatus. This rotatable element is in effect a bowl or vessel whose inner wall is provided with a novel arrangement of passages for the introduction and maintenance of the desired fluid current and for the accumulation and discharge of the solid particles of relatively high specific gravity. The inner wall of the rotatable vessel or bowl has a plurality of V-shaped riffles formed by the annular members 16 and 25. The solid particles undergoing separation or concentration accumulate in these V-shaped riffles and form a bed of solid particles as indicated by *b* in Fig. 2 of the drawings. The internal diameter of the rotatable bowl or vessel increases gradually and slightly from the bottom towards the top, whereby the mixture of solid particles to be separated or concentrated (fed into the bottom of the bowl through the feed pipe 32) tends to move up the inner wall of the bowl in response to the centrifugal action occasioned by the rotation of the bowl.

The operation of the apparatus illustrated in the accompanying drawings is substantially as follows:

Power is supplied to the drive shaft 13 and the rotatable element or bowl of the apparatus is rotated at an appropriate speed to develop the desired centrifugal action. Mercury, or other appropriate liquid of

high specific gravity in predetermined quantity is supplied to each of the aforementioned V-shaped riffles by means of the pipes 34 and the cooperating grooves 33 in the manifold 23. The material to be separated or concentrated, such as an ore or a slime, in the form of a pulp, is continuously fed into the bottom of the bowl through the central feed pipe 32 and is carried by centrifugal force up the inner surface of the rotating element, thereby forming in the V-shaped riffles a bed of ore constituents (*b* Fig. 2). A fluid, preferably water, is introduced in any appropriate manner into the distributing manifold 23 and is thereupon distributed to each of the chambers 20 in each annular member 16. The mercury, being heavier than any of the ore constituents occupies the outer portion of each V-shaped riffle, as indicated generally by the shading *a* in Fig. 2. The water, or other fluid, in the chambers 20, by virtue of its centrifugal and hydraulic head, flows through the relatively small holes 24 into the passages 28 and thence through the bed of the ore constituents in the V-shaped riffles. This flow of water maintains the bed of ore constituents in a more or less mobile condition, thus permitting the particles of heavy minerals to displace particles of lighter minerals and also permitting the particles of heavy minerals to progress towards the mercury seal at the apex of the U formed by the passages 27 and 28.

As the quantity of heavy mineral particles accumulates at the apex of the V-shaped riffles and in the passages 28, the pressure of these heavy mineral particles due to centrifugal force becomes sufficient to force the mercury to and slightly beyond the outer extremity of the upper horizontal edge of the annular member 25. A portion of the heavy mineral particles is thereby forced into the passage 27 and gradually progresses through this passage into the discharge compartments 29, from whence the heavy mineral particles are discharged by centrifugal action into the respective launders 30.

The lighter mineral particles flow with the current along the passage 28, in a direction opposite to the direction of the centrifugal action. The velocity of flow of the liquid current in the passage 28 is such as to overcome the effect of the centrifugal action on the solid particles of lower specific gravity but insufficient to overcome the effect of the centrifugal action on the solid particles of higher specific gravity. As a result the particles of lower specific gravity pass along with the fluid current and are carried up the inner wall of the rotating element or bowl. At each V-shaped riffle a concentrating or separating action takes place, and the ore or other ma-

terial progressing towards the top of the rotating element or bowl becomes gradually depleted of particles of heavy minerals. The tailings are discharged from the apparatus, by centrifugal force, over the top of the uppermost annular member 16 into the tailings launder or hopper 35.

- The **U** formed by the passages 27 and 28 functions as a seal for regulating and controlling the discharge of the solids of higher specific gravity. It will be observed that the passages 27 and 28 are so related that the effect of centrifugal action tends to force the solid particles towards the bottom 15 of the **U** formed by these passages. In other words, the passages 27 and 28 constitute in effect a two-part discharge passage, in one part of which the effect of the centrifugal action is substantially opposite in direction 20 to the effect of the centrifugal action in the other part whereby the discharge of solids from this two-part passage is regulated by the balancing of the effects of the centrifugal action in the two parts thereof. 25 When the effect of the centrifugal action on the particles in the passage 28 overcomes and over-powers the effect of the centrifugal action on the particles in the passage 27, then some of the particles in the passage 30 27 are forced out of this passage into the compartment 29 and are thrown therefrom by the centrifugal action into one of the launders 30.

The mercury seal in the passages 27 and 35 28 may be adjusted so as to automatically discharge from each riffle a product or concentrate of predetermined density or grade. Thus, the quantity of mercury in each of the two-part passages 27-28 may be independently controlled and adjusted so as to obtain a product or concentrate of high density or high grade in the lower riffles and a product or concentrate of lower density or lower grade in the upper riffles. In this 40 manner the operation of the apparatus can be controlled and minimum loss of values in the tailings insured. The use of mercury, or similar fluid seal, at the apex of the **V**-shaped riffles is not absolutely essential, but I have found the mercury seal of 45 particular advantage as a fluid base so that the balance of pressures in the **V**-shaped riffles will not be obstructed by packed solids.

The flow of water may be independently 50 regulated in each riffle. As a result of the **V**-shape of the riffles, the velocity of flow of the fluid current and the consequent sorting action is a maximum at the apex of the riffle and a minimum at the inner surface of 55 the bed of solid particles (indicated generally in Fig. 2 by *b*). In this manner the concentrate or heavy mineral particles are effectively cleaned before their discharge 60 without causing sufficient flow to carry values past the riffle. The water may be

supplied continuously or intermittently at short intervals, thus producing a pulsating flow as in a jig.

I claim:

1. The improvement in the method of 70 separating finely divided solids of different densities by centrifugal action which comprises discharging the solids of higher specific gravity through a discharge path of such character that centrifugal force acting 75 upon the accumulating solids of higher specific gravity effects a substantially continuous movement of such solids through a liquid seal operatively maintained in the discharge path by centrifugal action, and 80 maintaining said accumulating solids of higher specific gravity in a substantially mobile condition by the action of a fluid other than the sealing liquid which flows opposite in effect to the action of centrifugal force upon said accumulating solids. 85

2. The method of separating finely divided solids of different densities which comprises subjecting a mixture of such solid to centrifugal action and a fluid which 90 flows opposite in effect to the action of centrifugal force whereby solids of higher specific gravity are carried along by the centrifugal action against the fluid while solids of lower specific gravity are carried 95 along by the fluid to an appropriate discharge, and discharging the solids of higher specific gravity through a discharge path of such character that centrifugal force acting 100 upon the accumulating solids of higher specific gravity effects a substantially continuous movement of such solids through a liquid other than the fluid which carries along solids of lower specific gravity, which is operatively maintained as a liquid seal 105 in the discharge bath by centrifugal action.

3. The method of separating finely divided solids of different densities which comprises subjecting a mixture of such solids to centrifugal action and a fluid which flows 110 opposite in effect to the action of centrifugal force whereby solids of higher specific gravity are carried along by the centrifugal action against the fluid while solids of lower specific gravity are carried along by the 115 fluid to an appropriate discharge, and discharging the solids of higher specific gravity through a two-part passage and a liquid operatively maintained in the passage other than the fluid which carries along solids of lower specific gravity, the effect of the centrifugal action in one part of the two part passage being opposed by the effect of the centrifugal action in the other part whereby the discharge of the solids from said passage is regulated by the balancing of the effects of the centrifugal actions in the two parts of the passage. 125

4. The method of separating finely divided solids of different densities which 130

- comprises subjecting a mixture of such solids to the resulting effect of centrifugal action and an opposing fluid current whereby solids of higher specific gravity are carried 5 along by the centrifugal action against the fluid current while solids of lower specific gravity are carried along by the fluid current to an appropriate discharge, and discharging the solids of higher specific gravity through 10 a mercury seal contained in a two-part passage in one part of which the effect of the centrifugal action is substantially opposed to the effect of the centrifugal action in the other part whereby the discharge of the 15 solids by said mercury seal is regulated by the balancing of the effects of the centrifugal actions in the two parts of the passage.
5. The method of separating finely divided solids of different densities which comprises subjecting the mixture of such solids to the action of centrifugal force while suspended in a liquid flowing in a direction substantially opposite to the direction of the centrifugal force and at such a velocity as to 20 overcome the effect of the centrifugal action on the solids of lower specific gravity while insufficient to overcome the effect of the centrifugal action on solids of higher specific 25 gravity, maintaining an accumulation of 30 solids of the centrifugal separation, subjecting said accumulation of solids to the cleaning action of the liquid flowing in a direction opposite to the direction of the centrifugal force, and discharging the solids of higher 35 specific gravity through a two-part passage in one part of which the effect of the centrifugal action is opposed by the effect of the centrifugal action in the other part, whereby the discharge of the solids from said passage 40 is regulated by the balancing of the effects of the centrifugal actions in the two parts of the passage.
6. An apparatus for the separation of finely divided solids of different densities comprising a rotatable bowl having a plurality of superposed V-shaped riffles on its inner wall, a series of U-shaped discharge passages having one arm communicating with the apex of one of said riffles and the other arm communicating with a discharge compartment, means for causing a fluid current to flow inwardly from the apex of each of said riffles, and means in the other arm actuated by the action of centrifugal force 45 for regulating the discharge of separated solids.
7. In an apparatus of the character described, a rotatable drum comprising a chamber for the reception of the material to be treated, means for introducing the material to be treated, means for introducing a supply of liquid to the outer limits of the concentrating chamber, an annular channel 50 connected with the outer limit of the concentrating chamber and forming with it a U for discharging automatically a product by the operation of balanced forces, and a mercury seal in the U.
8. In an apparatus of the character described, a rotatable drum comprising a series of annular V-shaped riffles for the reception of the material to be treated, means for introducing a supply of liquid to the apex of the riffles, an annular channel connected to the apex of each riffle and forming with it an automatic discharging U, a mercury seal in the U forming a fluid base for the operation of the balanced discharging forces.
9. An apparatus for the concentration of ores comprising a vessel adapted to contain a finely divided ore suspended in a liquid, a discharge passage in the vessel, means for directing the ore constituents toward the discharge passage by centrifugal action, a fluid conduit associated with said discharge passage and adapted to direct a flow of fluid into the vessel in a direction opposed to said centrifugal action to thereby segregate the desired heavy ore constituents near the discharge passage and to remove therefrom the remaining ore constituents, means for discharging a portion of said desired heavy ore constituents in response to said centrifugal action and for permitting cleaning of the remaining portion of the heavy ore constituents by the action of the fluid flowing in a direction opposed to the centrifugal action, and means for removing said remaining ore constituents by the flow of said fluid.
10. An apparatus for the concentration of ores comprising a vessel adapted to contain a finely divided ore suspended in a liquid, a discharge passage in the vessel, means for directing the ore constituents toward the discharge passage by centrifugal action, a fluid conduit associated with said discharge passage and adapted to direct a flow of fluid into the vessel in a direction opposed to said centrifugal action to thereby segregate the desired heavy ore constituents near the discharge passage and to remove therefrom the remaining ore constituents, means for maintaining an accumulation of a predetermined quantity of the desired heavy ore constituents near said discharge passage and permitting discharge of an excess of the desired ore constituents by centrifugal action, and means for removing said remaining ore constituents by the flow of said fluid.
11. An apparatus for the concentration of ores comprising a vessel adapted to contain a finely divided ore suspended in a liquid, an annular discharge passage extending away from and then toward the interior of the vessel, means for directing the ore constituents toward the discharge passage by centrifugal action, a fluid conduit associated with said discharge passage and adapted to

- direct a flow of fluid into the vessel in a direction opposed to said centrifugal action to thereby segregate the desired heavy ore constituents near the discharge passage and remove therefrom the remaining ore constituents, means for maintaining in said discharge passage a liquid of high specific gravity in such quantity as to maintain an accumulation of a predetermined quantity of said heavy ore constituents and permit discharge of an excess of the desired heavy ore constituents by centrifugal action, and means for removing said remaining ore constituents by the flow of said liquid.
- 5 13. An apparatus for the concentration of ores comprising a vessel adapted to contain a finely divided ore suspended in a liquid, an annular discharge passage extending outward and then toward the interior of the vessel, means for directing the ore constituents toward the discharge passage by centrifugal action, a liquid conduit communicating with the outward extending portion of the discharge passage for introducing liquid in a direction opposed to the travel of the ore constituents to thereby segregate the desired heavy ore constituents near the discharge passage and remove therefrom the remaining ore constituents, means for maintaining in said discharge passage a liquid of high specific gravity in such quantity as to maintain an accumulation of a predetermined quantity of said heavy ore constituents and permit discharge of an excess of the desired heavy ore constituents by centrifugal action, and means for removing said remaining ore constituents by the flow of said liquid.
- 10 14. An apparatus for the concentration of ores comprising a vessel adapted to contain a finely divided ore suspended in a liquid, an annular discharge passage extending away from and then toward the interior of the vessel, means for directing the ore constituents toward the discharge outlet by centrifugal action, means for causing a flow of the liquid in a direction opposed to said centrifugal action to thereby segregate the heavy ore constituents near the discharge passage and to remove therefrom the remaining ore constituents means for maintaining in said discharge passage a liquid of high specific gravity in such quantity as to maintain an accumulation of a predetermined quantity of said heavy ore constituents and permit
- 15 15. 12. An apparatus for the concentration of ores comprising a vessel adapted to contain a finely divided ore suspended in a liquid, an annular discharge passage extending away from and then toward the interior of the vessel, means for directing the ore constituents toward the discharge outlet by centrifugal action, means for causing a flow of the liquid in a direction opposed to said centrifugal action to thereby segregate the heavy ore constituents near the discharge passage and to remove therefrom the remaining ore constituents means for maintaining in said discharge passage a liquid of high specific gravity in such quantity as to maintain an accumulation of a predetermined quantity of said heavy ore constituents and permit
- 20 16. An apparatus for the concentration of ores comprising a vessel adapted to contain a finely divided ore suspended in a liquid, an annular discharge passage extending away from and then toward the interior of the vessel, means for directing the ore constituents toward the discharge outlet by centrifugal action, means for causing a flow of the liquid in a direction opposed to said centrifugal action to thereby segregate the heavy ore constituents near the discharge passage and to remove therefrom the remaining ore constituents means for maintaining in said discharge passage a liquid of high specific gravity in such quantity as to maintain an accumulation of a predetermined quantity of said heavy ore constituents and permit
- 25 17. An apparatus for the concentration of ores comprising a vessel adapted to contain a finely divided ore suspended in a liquid, an annular discharge passage extending away from and then toward the interior of the vessel, means for directing the ore constituents toward the discharge outlet by centrifugal action, means for causing a flow of the liquid in a direction opposed to said centrifugal action to thereby segregate the heavy ore constituents near the discharge passage and to remove therefrom the remaining ore constituents means for maintaining in said discharge passage a liquid of high specific gravity in such quantity as to maintain an accumulation of a predetermined quantity of said heavy ore constituents and permit
- 30 18. An apparatus for the concentration of ores comprising a vessel adapted to contain a finely divided ore suspended in a liquid, an annular discharge passage extending away from and then toward the interior of the vessel, means for directing the ore constituents toward the discharge outlet by centrifugal action, means for causing a flow of the liquid in a direction opposed to said centrifugal action to thereby segregate the heavy ore constituents near the discharge passage and to remove therefrom the remaining ore constituents means for maintaining in said discharge passage a liquid of high specific gravity in such quantity as to maintain an accumulation of a predetermined quantity of said heavy ore constituents and permit

35 40 45 50 55 60

In testimony whereof I affix my signature.

HENRY ALFRED DOERNER.